

Patented Feb. 20, 1923.

1,446,301

# UNITED STATES PATENT OFFICE.

HORACE JAMES HEGAN, OF COVENTRY, ENGLAND, ASSIGNOR TO COURTAULDS  
LIMITED, OF LONDON, ENGLAND.

## MANUFACTURE OF THREADS, FILAMENTS, AND THE LIKE OF CELLULOSE.

No Drawing.

Application filed March 31, 1922. Serial No. 543,530.

To all whom it may concern:

Be it known that I, HORACE JAMES HEGAN, a subject of the King of Great Britain, residing at Spring House, Radford Road, in 5 the city of Coventry, England, have invented new and useful Improvements in or Connected with the Manufacture of Threads, Filaments, and the like of Cellulose, of which the following is a specification.

10 This invention relates to the manufacture of threads, filaments, and the like, from viscose, in the preparation of which cotton has been used as the source of cellulose, including under the term "cotton" any suitable 15 kind of cotton, such, for example, as long-fibred cotton, or cotton with short fibres such as is obtained from cotton-seed hulls.

In the production of threads, filaments, and the like, of cellulose, by projecting the 20 said viscose through small orifices into a bath having an acid reaction, such, for instance, as a bath containing sulphuric acid and a sulphate with, or without, the addition of other suitable compound, or compounds, such, for instance, as glucose and a 25 zinc salt, there is generally a tendency, especially in the spinning of fine filaments, for one, or more, of the threads, filaments, or the like, to break, and for globules of viscose, 30 more, or less, coagulated, to form at the nozzle and pass up with the thread onto the winding apparatus. This causes unevenness of the resulting thread, and such unevenness is generally not desirable.

35 According to the present invention the tendency to break and form such globules is reduced by introducing into the viscose, either as such, or during the preparation thereof, a substance, which lowers, or substances which lower, the surface tension of 40 the viscose in comparison with the spinning bath employed, such substance, or substances, having either in itself, or themselves, or by reason of the small quantity 45 used, practically no setting action on the viscose, and neither it, or they, nor its, or their, decomposition products having any injurious, or objectionable, effect upon the threads, filaments, or the like.

50 Provided that the viscose, when ready for conversion into threads and the like, contains a substance, or substances, which will lower the surface tension of the viscose, such substance, or substances, may be added directly to the viscose, or in any suitable man-

ner to any one, or more, of the ingredients employed in the ultimate preparation of the viscose, or of any of the intermediate products, although it is preferred to prepare the alkali cellulose in the absence of such substance, or substances. 60

I give the following as an example of how this invention may be performed, without restricting the invention to this example. Two parts by weight of sodium oleate are 65 introduced into the materials from which ten thousand parts by weight of viscose are prepared, the sodium oleate being preferably dissolved in the water, or dilute alkali employed for the solution of the cellulose 70 xanthate. The viscose, after being prepared, and after having attained the desired ripeness, is passed through a nozzle containing orifices of the desired diameter, into a bath containing sulphuric acid, sodium sulphate, and glucose together with a 75 small quantity of a zinc salt.

What I claim is:—

1. In the manufacture of threads, filaments, and the like, from viscose prepared 80 from cotton, the introduction into the setting bath of cotton-viscose containing a substance which will lower the surface tension of the viscose.

2. In the manufacture of threads, filaments, and the like, from viscose prepared from cotton, the introduction into the setting bath of cotton-viscose containing sodium oleate. 85

3. For use in the manufacture of threads, 90 filaments, and the like, viscose prepared from cotton and containing sodium oleate in approximately the proportion of two parts by weight of sodium oleate to ten thousand parts by weight of viscose. 95

4. In the preparation of viscose from cotton, the step of dissolving the cellulose xanthate in a fluid containing sodium oleate, the said sodium oleate being present in approximately the proportion of two parts by weight to ten thousand parts by weight of viscose. 100

In testimony whereof I have signed my name to this specification in the presence of two subscribing witnesses.

HORACE JAMES HEGAN.

Witnesses:

WILLIAM HENRY STOKES,  
JOHN ALEXANDER LLOYD.